

## UNITED STATES PATENT OFFICE

2,197,611

## METHOD OF PRODUCING PROTECTIVE COATINGS ON MAGNESIUM AND THE ALLOYS THEREOF

Johannes Fischer, Berlin - Siemensstadt, and Werner Richter, Berlin, Germany, assignors to Siemens & Halske, Aktiengesellschaft, Siemensstadt, near Berlin, Germany, a corporation of Germany

No Drawing. Application May 20, 1936, Serial No. 80,908. In Germany June 1, 1935

6 Claims. (Cl. 204—1)

Our invention relates to a method for producing protective coatings on magnesium and the alloys thereof, hereinafter referred to as magnesium.

5 It is well known in the art to produce coatings on magnesium with the aid of an electric current which protect this valuable light metal against corrosive influences of any kind. This may, for instance, be accomplished by electrolysis of fused fluoride electrolytes. The difficulties and disadvantages presented in the treatment of baths containing a fused electrolyte are so well known that they need not be dealt with here. Of course, attempts have also been 10 made to replace the fused electrolyte by an electrolyte which may be employed at normal temperature.

Experiments to produce protective coating on magnesium in an aqueous solution led to the 20 well-known rule of utilizing baths containing alkali hydroxides or alkaline-earth hydroxides. Experience has shown that this rule cannot be applied under certain circumstances. If, for instance, an electrolyte is used which contains 25 only caustic soda no coating of any practical value can be produced. It may even happen that the metallic surface becomes very often pitted.

Accordingly experiments have been carried out 30 to substitute other alkaline substances for the mordant alkali. In this connection the experiments with carbonate of alkali as electrolytic component did not give any satisfactory results. The same applies to the electrolysis in 35 cyanide baths.

However, the experiments have surprisingly shown that the electrolyte must contain according to the invention at least three components in order to attain satisfactory coatings that may 40 be reproduced at will. The three electrolytic components necessary according to the invention must be taken from the groups of compounds which present a certain chemical affinity with one another.

45 To the first group belong besides the alkali metal hydroxides, which are preferably employed, also the alkaline-earth hydroxides and the aqueous solution of ammonia. The second group comprises water soluble carbonates, silicates and 50 borates; also the salts of the polyboric acids may be employed. Finally the third group includes cyanides, thiocyanides and cyanates.

The electrolytes composed according to the invention of at least three substances, one from each of the three groups, produce when anodi-

cally treating magnesium very satisfactory protective layers which, when coated with inorganic or organic sealing means render the metallic supports highly resistant to corrosion. As sealing means varnish, grease, oil, wax, colloidal 5 hydroxide, silica gel, etc., may be employed.

The porosity of the novel layers enables the application of a color which may be desirable for certain purposes. Instead of the dye solutions any other filling material solutions may, 10 of course, be utilized for treating the electrolytically prepared objects of magnesium. It should be considered that the porosity of the novel layers decreases with time. Experiments have shown that the newly produced protective coatings present a considerably greater adsorptive power with respect to coloring substances of any kind than seasoned protective coatings. This fact renders it possible to regulate the depth of color. As coloring substances all organic dye 20 solutions may be utilized as well as colored inorganic substances precipitated in the layer.

The voltage is preferably taken as 16 volts. However, good results may also be attained with a gradual change in voltage. Thus a coating was 25 produced at a voltage of 16 volts and then the coating was strengthened at 60 or 110 volts. The strengthening of the coating is possible owing to the greater residual current resulting from the higher voltages. Finally also gradually 30 increasing voltages may under certain circumstances be employed; for instance, by gradually increasing the voltage from 1 volt to 60 or 110 volts, while maintaining the intensity of the current constant.

35 The temperature during the treatment is preferably chosen between 20° and 25° centigrade, since at a higher temperature a pitting occurs. It is, therefore, necessary to cool the object to be treated during the passage of the current. 40 At temperatures which lie considerably below 20° the current is blocked too quickly so that the formation of a good thick absorbing layer is prevented. This phenomenon is due to the fact that the residual current at low temperatures becomes considerably weaker. The current density decreases by 80% suddenly during the first seconds of the treating period. It is kept at this low value preferably for 60 minutes. 45 After this treating period the electrolytical process may be considered as terminated. In particular cases in which colored coatings are desired the objects are then treated with the dye solution and finally they are sealed; for instance, 50 55

varnished so as to protect them against corrosion.

While the three above-mentioned groups of substances must be present in the electrolyte further admixtures from a fourth group may be employed when composing the electrolyte which produce then a better coating. This fourth group of substances includes the water soluble sulphates, nitrates, phosphates, halogenides, 10 halogenates, fluosilicates, chromates, tungstates, etc.

As to the concentration to be used a great advantage is obtained from the industrial point of view, since the so-called degreasing baths for 15 electroplating obtainable on the market present the desired concentration for the novel method. Soda, for instance, may be used with success in a 5% solution, pure caustic soda in a 6% solution of NaOH and potassium cyanide in a 2% solution of KCN.

The cations, particularly the alkalies, may be replaced by one another or uniformly chosen from all three groups; only ammonium forms an exception, since a very bad coating was attained in connection with ammonium compounds.

*Example 1.*—In an aqueous electrolyte containing 5% of NaOH, 5% of Na<sub>2</sub>CO<sub>3</sub>, 2% of KCN and 0.1% of Na<sub>2</sub>WO<sub>4</sub> a sheet metal consisting of an alloy of magnesium was subjected 30 anodically at a temperature of 20° C. to the action of the current. At a voltage of 16 volt a current density of 5 amp./dm.<sup>2</sup> was attained in the first moment and this decreased to 1 amp./dm.<sup>2</sup> within the following 30 seconds. The 35 current treatment lasted an hour. The sheet metal provided with the fresh layer was dipped into a dye solution and then coated and varnished. The layer thus produced was extremely tight and uniformly colored.

*Example 2.*—Instead of the sodium tungstate employed in Example 1 as electrolytic admixture, potassium iodide, potassium chromate, sodium chloride, potassium chlorate, potassium nitrate, sodium silicate and sodium sulphate were alternately used in succession as electrolytic admixture at a concentration of 0.1%. Particularly good absorbing layers were obtained when admixing potassium iodide, potassium chlorate and potassium nitrate. Experiments have shown 45 that an admixture of potassium iodide and sodium silicate caused a pitting at the surface of the liquid. In the last-mentioned example a relatively slight porosity of the coating resulted.

*Example 3.*—The method according to the invention was carried out without admixing a substance of the fourth group. In this case instead of 5% of Na<sub>2</sub>CO<sub>3</sub>, 5% of borax (Na<sub>2</sub>B<sub>4</sub>O<sub>7</sub>) or 5% of water glass (Na<sub>2</sub>SiO<sub>3</sub>) was used. The electrolyte consisting of potash lye, soda and potassium cyanide gave without any admixture 55 excellent results which, however, could be further improved by substituting borax for soda; that is to say the porosity of the coating is improved. Even without the admixture of a substance of the fourth group the electrolytes containing water glass produced a layer of a slighter porosity.

*Example 4.*—Protective layers were produced in an electrolyte which contained 2% of KCNS and 70 2% of KCNO instead of 2% of KCN. In the first case a very hard coating which was substantially free of pores was produced, whereas when using KCNO as electrolytic component a good average result was obtained.

75 *Example 5.*—Finally the same cation was em-

ployed for all components. An experiment was carried out with 5% of KOH, 5% of K<sub>2</sub>CO<sub>3</sub>, 2% of KCN and 0.1% of K<sub>2</sub>SO<sub>4</sub>. The absorptive power of the layer thus produced was above average.

The expression "the simple cyanides, thiocyanides and cyanates of the alkali metals" as used in the following claims, is intended to exclude compounds such as the so-called complex, compound or double cyanides of the alkali metal cyanides and cyanides of the heavy metals.

We claim as our invention:

1. The method of producing non-metallic protective coatings on magnesium, which comprises anodically treating the magnesium in an aqueous solution of a mixture consisting substantially of hydroxide selected from the group consisting of alkali metal hydroxides, alkaline earth hydroxides and aqueous ammonia, and salt selected from the group consisting of water soluble carbonates, silicates and borates, and salt selected from the group consisting of the simple cyanides, thiocyanides and cyanates of the alkali metals.

2. The method of producing non-metallic protective coatings on magnesium, which comprises anodically treating the magnesium at a temperature between 20 and 25° C. in an aqueous solution of a mixture consisting substantially of hydroxide selected from the group consisting of alkali metal hydroxides, alkaline earth hydroxides and aqueous ammonia, and salt selected from the group consisting of water soluble carbonates, silicates and borates, and salt selected from the group consisting of the simple cyanides, thiocyanides and cyanates of the alkali metals.

3. The method of producing non-metallic protective coatings on magnesium, which comprises anodically treating the magnesium at between 1 and 110 volts at a temperature of about 20 to 25° C. in an aqueous solution of a mixture consisting substantially of hydroxide selected from the group consisting of alkali metal hydroxides, alkaline earth hydroxides and aqueous ammonia, and salt selected from the group consisting of water soluble carbonates, silicates and borates, and salt selected from the group consisting of the simple cyanides, thiocyanides and cyanates of the alkali metals.

4. The method of producing non-metallic protective coatings on magnesium, which comprises anodically treating the magnesium at about 16 volts in an aqueous solution of a mixture consisting substantially of hydroxide selected from the group consisting of alkali metal hydroxides, alkaline earth hydroxides and aqueous ammonia, and salt selected from the group consisting of water soluble carbonates, silicates and borates, and salt selected from the group consisting of the simple cyanides, thiocyanides and cyanates of the alkali metals.

5. The method of producing non-metallic protective coatings on magnesium, which comprises anodically treating the magnesium at a voltage increasing from less than 16 volts to at least about 60 volts in an aqueous solution of a mixture consisting substantially of hydroxide selected from the group consisting of alkali metal hydroxides, alkaline earth hydroxides and aqueous ammonia, and salt selected from the group consisting of water soluble carbonates, silicates and borates, and salt selected from the group consisting of the simple cyanides, thiocyanides and cyanates of the alkali metals.

6. The method of producing non-metallic pro-

5 tective coatings on magnesium, which comprises anodically treating the magnesium in an aqueous solution of a mixture consisting substantially of hydroxide selected from the group consisting of alkali metal hydroxides, alkaline earth hydroxides and aqueous ammonia, salt selected from the group consisting of water soluble carbonates, silicates and borates, salt selected from the group consisting of the simple cyanides, thiocyanides

and cyanates of the alkali metals, and a small but effective amount, sufficient to improve the porosity of the coating, of a water soluble ingredient consisting of an alkali metal salt of a highly dissociated acid, the concentration of said latter ingredient being lower than that of said three groups. 5

JOHANNES FISCHER.  
WERNER RICHTER.